

(No Model.)

2 Sheets—Sheet 1.

W. F. M. McCARTY.

METHOD OF PRODUCING STEEL DIRECT FROM ORE.

No. 404,723.

Patented June 4, 1889.



WITNESSES  
F. L. Ourand.  
A. M. Mahan

INVENTOR  
W. F. M. McCarty  
G. S. Gisalang  
Attorney

(No Model.)

2 Sheets—Sheet 2.

W. F. M. McCARTY.

METHOD OF PRODUCING STEEL DIRECT FROM ORE.

No. 404,723.

Patented June 4, 1889.

Fig. 2.

Fig. 3.



WITNESSES

F. L. Ourand.

Alex. Mahon

INVENTOR

W. F. M. McCarty  
J. S. McFarland  
Attorney

# UNITED STATES PATENT OFFICE.

WILLIAM F. M. McCARTY, OF HAGERSTOWN, MARYLAND, ASSIGNOR, BY DIRECT AND MESNE ASSIGNMENTS, OF PART TO JANE LOGAN, OF SAME PLACE, CATHERINE EISHON, OF PHILADELPHIA, PENNSYLVANIA, AND HEMAN D. WALLBRIDGE.

## METHOD OF PRODUCING STEEL DIRECT FROM ORE.

SPECIFICATION forming part of Letters Patent No. 404,723, dated June 4, 1889.

Application filed February 26, 1889. Serial No. 301,297. (No model.)

*To all whom it may concern:*

Be it known that I, WILLIAM F. M. McCARTY, a citizen of the United States, residing at Hagerstown, in the county of Washington 5 and State of Maryland, have invented new and useful Improvements in the Method of Producing Steel Direct from Ores; and I do hereby declare the following to be a full, clear, and exact description of said invention, reference being had to the accompanying drawings, and to the letters or figures of reference marked thereon, which form a part of this specification.

My invention consists in the process of producing steel direct from ore; and to obtain a 15 full understanding of the process it should be stated that heretofore it has been impossible to produce steel direct from the ore for many reasons, the principal one of which has been 20 to keep the mass of ore and fuel separate while being acted upon by the calorific energy of the burning fuel.

To carry out my process I have designed the apparatus as shown in the accompanying 25 drawings, in which—

Figure 1 is a transverse section of a blast-furnace, showing one manner of constructing the stack in which the bosh thereof is shown in spherical form and connected with converter through a narrow passage-way. Fig. 30 2 is a similar section of another manner of constructing the stack and converter, showing the vacuum-chamber also in section and the preferred relation of the air and gas-heater to the stack. Fig. 3 is a horizontal section through the line  $x-x$ , Fig. 2.

The stack may be of any usual or convenient construction provided at some distance from the lower end with an annular offset to 40 support the charge of fuel and ore introduced through the opening D near the top. Below the offset is what I term the "bosh" B of the stack which communicates through a central opening with the converter A below.

In Fig. 1 the bosh is made in spherical form and communicates with the producer through a contracted passage-way  $d$ , while in Fig. 2 said bosh is made in tapering cylindrical form, with its lower portion contracted to form 50 the passage-way between it and the converter.

The upper end of the stack has an outlet  $a$  for the gases and products of combustion, and has a side flue  $P$ , controlled by a damper  $a'$ , which can direct the products of combustion either out at the top or into the side flues  $P$ , 55 the latter communicating with the down-comer flue or pipe  $P'$ , leading to the air-heater or hot-blast producer L. On the opposite side of the stack is shown a heater M, for heating the gases to be used in working the charge. 60 The converter below the bosh of the stack communicates through a valve-pipe  $m$  with a second converter or gas-extractor J, this pipe opening into the converter A at some distance from the bottom, in order that the 65 molten metal at the upper part of the converter A may flow out as it is treated into the gas extractor or converter J. The receiver J communicates through a suitable opening  $j$  with a vacuum-chamber K, or some equivalent device for producing a vacuum.

At different heights in the stack I provide suitable tuyeres for the introduction into the charge at different zones of gas or gases, or combined air and gas, as hereinafter described. The uppermost set E of tuyeres I prefer to arrange at such a point that the gases introduced thereby may pass directly into the upper part of the charge of ore while the next lower set of tuyeres F is at some distance 80 above the offset  $v$ . A third set of tuyeres G are introduced just below the offset  $v$ , and another set H into the bosh of the stack, and a final set into the converter A.

Formed in the internal wall of the stack, 85 and projecting therefrom, are a series of shelves inclining inward with their inner edges overhanging the ones next below, as shown in Fig. 2, or the stack is provided with a central wall having shelves projecting therefrom alternating with those projecting from the wall of the stack, the edges of each overlapping the others, for a purpose hereinafter referred to.

In carrying out my process, after the ore 95 has been sorted it is cracked up in sizes suitable for the crusher, and after being crushed it is passed to the ore-mill to be reduced to powder, when a proper charge thereof with sufficient flux and coke or other fuel to start 100

the operation is introduced into the stack through the charging-opening D and falls upon the shelving. Atmospheric air, with carbonic oxide and hydrogen, is then introduced 5 through the tuyeres E and ignited to start the fire. Hydrogen and carbonic oxide are next introduced through the tuyeres F into the body of the charge, and also at H, if desired, until the mass is in a state of combustion. I then introduce into the upper part of the charge through the tuyeres E pure hydrogen gas, to thoroughly deoxidize and reduce the ore by the removal of oxygen and sulphur contained therein, leaving the iron 5 in a free metallic state or spongy mass.

Although I have said that carbonic oxide should be introduced through the intermediate tuyeres F G II with the hydrogen, I wish it to be understood that the necessary 5 o carbon may be there introduced with the hydrogen by other means. For instance, powdered carbon or liquid hydrocarbon oil or carbonic oxide may be introduced with the hydrogen; but I prefer carbonic oxide.

5 The relative proportions of hydrogen and carbon introduced through the intermediate tuyeres will vary to some extent with the character of the ores under treatment. As soon as the metal begins to fuse under the intense heat produced by the introduction of the gases and air at different zones, as above described, the molten metal will commence to fall down through the bosh into the converter A, when the pure hydrogen and superheated 5 air are turned on through the tuyeres I to decarbonize and purify the molten metal, which has been partly acted upon by gases introduced through the tuyeres II in its descent through the bosh B of the furnace.

o The oxygen of the air and the hydrogen introduced into the molten metal in the converter A produce an intense heat and remove the silicon and other impurities and a large portion of the carbon in the metal, and by 5 regulating these gases according to the nature of the ores under treatment a pure homogeneous steel will be produced.

In some instances where it is found that the molten metal in the converter A has not received sufficient carbon in its descent through the furnace the proper proportion of carbon in the form of finely-divided graphite spiegeleisen with cyanogen and air may be introduced through the tuyeres I.

5 When it is determined that the steel is of the desired quality, the valve in the outlet-pipe m is opened and the overflow of the metal takes place into the second receiver J. When this chamber has been filled with sufficient metal for the run, the valve in the pipe m is closed and connection with the vacuum-chamber is opened. This will insure the withdrawal from the molten mass of any

gases which may have remained therein. Homogenous steel is thus produced free from 65 the usual defects, such as blow-holes, honeycombs, or other faults.

The operation, as will be readily seen, can be made continuous by connecting the opening D with a hopper, which can be so arranged 70 as to govern the supply, so that a continuous fusion is going on automatically, the metal falling in the form of ore and flux intimately mixed from shelf to shelf of its own gravity, the shelves being arranged on a proper incline, and the material falling in a continuous 75 manner from shelf to shelf while being heated by the gaseous fuel.

Having now described my improved process and one means for carrying the same into effect, what I claim as my invention is—

1. The process which consists in introducing into a highly-heated charge of iron ore and flux hydrogen gas, and subsequently at different points into the charge hydrogen and 85 carbonaceous matter in a state of combustion in order to melt and subsequently carbonize the metal, substantially as set forth.

2. The process consisting in introducing into the highly-heated charge of iron ore and 90 flux hydrogen gas to reduce the ore, subsequently introducing hydrogen and carbonaceous matter with air at different points into the same charge to melt the metal, and finally introducing hydrogen and atmospheric air 95 with or without carbon into the molten metal to convert it into steel, substantially as set forth.

3. The process herein described of producing steel direct from the ore, said process consisting in first reducing the ore by introducing pure hydrogen into the charge of highly-heated ore and flux, then introducing hydrogen and carbonaceous matter with air to melt the metal, and subjecting the molten 105 metal in its passage from the stack to the converter to the action of hydrogen and carbonaceous matter, substantially as described.

4. The herein-described continuous process of producing steel direct from the ore, said 110 process consisting in first introducing hydrogen in the charge of highly-heated ore and flux to reduce the ore, then subjecting the charge to the action of hydrogen and carbonaceous material with air to melt the metal, 115 then subjecting the molten metal to the action of purifying gases and air, and finally subjecting the molten steel thus produced to the action of a vacuum, substantially as set forth.

In testimony whereof I affix my signature in 120 the presence of two subscribing witnesses.

WM. F. M. McCARTY.

Witnesses:

ALEX. MAHON,  
WARREN C. STONE.